

# UNITED STATES PATENT OFFICE.

CARL BOSCH, ALWIN MITTASCH, AND CHRISTOPH BECK, OF LUDWIGSHAFEN-ON-THE-RHINE, GERMANY, ASSIGNEES, BY MESNE ASSIGNMENTS, TO THE CHEMICAL FOUNDATION, INC., A CORPORATION OF DELAWARE.

## MANUFACTURE OF OXIDS OF NITROGEN.

1,379,387.

Specification of Letters Patent. Patented May 24, 1921.

No Drawing.

Application filed February 25, 1915. Serial No. 10,627.

To all whom it may concern:

Be it known that we, CARL BOSCH, ALWIN MITTASCH, and CHRISTOPH BECK, citizens of the German Empire, residing at Ludwigshafen-on-the-Rhine, Germany, have invented new and useful Improvements in the Manufacture of Oxids of Nitrogen, of which the following is a specification.

It has been proposed to convert ammonia into oxids of nitrogen, or nitric acid, by passing ammonia together with an oxygen-containing gas, such as air or oxygen, at a raised temperature, over oxids of the metals of the iron group, but the results hitherto obtained have varied considerably and have been generally unsatisfactory.

We have found that we may carry out the manufacture of oxids of nitrogen by the catalytic oxidation of ammonia in a regular manner and with good yields by employing the oxid, or oxids, or mixtures of the oxids of the metals of the iron group, in separate pieces, or lumps, of which a sufficiently deep layer should be used. The size and shape of the pieces, or lumps, may vary, for instance, according to the width of the contact tube, or furnace, and it is often advantageous to heat the pieces, or lumps, or otherwise treat them before use so that no sintering, or local fusion, of the surface, with consequent formation of irregular spaces, takes place in the contact tube, or furnace. The pieces, or lumps, may preferably contain 30 per cent. or more of an oxid of a metal of the iron group or of a mixture of more than one of the said oxids and may be dense or porous, it being particularly advantageous in the former case to employ pieces, or lumps, produced by breaking up a mass obtained by allowing an oxidized melt to solidify. Or a suitable stable contact mass may be obtained by burning pure iron powder in a current of oxygen, so that a molten oxid is produced, and then breaking up the solidified mass into pieces, or lumps, of about the size of a pea, or millet or still larger. Use can, however, be made of other pieces, or lumps, such, for instance, as those obtained by breaking up sufficiently pure

ores. If desired, the pieces, or lumps, may be 50 porous, in order to facilitate the passage of the gases. Suitable porous contact masses can, for instance, be obtained by calcining decomposable salts, such as nitrates, and then breaking up the product; or hydrox- 55 60 65 70 75 80 85 90 95 ies, or other compounds, may be employed which are directly made into pieces, or lumps, of any suitable shape. Thus, for instance, a hydroxid of iron, of manganese, of chromium, or of uranium, or a mixture of such hydroxids, may be precipitated by ammonia, or ammonium carbonate, or soda, from a solution of a suitable salt, or suitable salts, for instance, nitrates, or sulfates, and, after being well washed and sufficiently de- 60 65 70 75 80 85 90 95 prived of water, the precipitate can be pressed to form pieces, or lumps; or a part of the washed hydroxid may be dried, at say about 250° centigrade, then intimately mixed with the remaining damp portion and made into pieces, or lumps, of any desired shape such, for instance, as cubes, cylinders, spheres, or the like. The pieces, or lumps, are preferably heated, to say from 500°, to 700°, centigrade before being used. We may also start from metallic pieces, or lumps, for instance, from a number of small spheres, or the like, of pure iron, which may be placed in the contact tube, or furnace, either without treatment, or after being superficially oxidized.

The length of the layer of the contact mass, and the velocity of the gases, and the temperature employed, may vary considerably. Compounds which injuriously affect the catalytic action should not be present in the contact mass or in the gases, and it is generally advantageous to avoid sulfur, phosphorus, silica and alkali, especially in large quantities. On the other hand, indifferent bodies, or compounds, which promote their activity may be added to the metallic oxid, or oxids.

We claim:

1. The process of producing oxids of nitrogen by passing a mixture of ammonia and an oxygen-containing gas at a raised temperature over a granulated catalyst con-

taining a molten and again solidified oxid of a metal of the iron group.

2. A process of producing oxides of nitrogen which comprises passing a mixture of ammonia and oxygen containing gas at an elevated temperature over a catalyst containing a molten and again solidified oxid of a metal of the iron group.

In testimony whereof we have hereunto

set our hands in the presence of two sub- 10  
scribing witnesses.

CARL BOSCH.

ALWIN MITTASCH.

CHRISTOPH BECK.

Witnesses:

ARTHUR DENONVILLE,  
JOHANNES FEHMEL.